

# UNITED STATES PATENT OFFICE.

OTTO RÖHM, OF DARMSTADT, GERMANY, ASSIGNEE TO RÖHM & HAAS, OF DARMSTADT,  
GERMANY.

## PROCESS OF DEGUMMING SILK.

1,186,440.

Specification of Letters Patent. Patented June 6, 1916.

No Drawing.

Application filed February 5, 1915. Serial No. 6,342.

To all whom it may concern:

Be it known that I, OTTO RÖHM, subject of the German Emperor, residing at Nos. 4-6 Weiterstädterstrasse, Darmstadt, German Empire, have invented new and useful Improvements in the Process of Degumming Silk; and I do hereby declare the following to be a full, clear, and exact description of the same.

10 My invention relates to improvements in the process of degumming silkworms' cocoons, waste silk, and the like. At present this process is carried out by putrefaction or by boiling the silk with soap. These 15 processes are objectionable. The putrefying process requires much time, and as it is a bacterial process its progress cannot well be controlled, and it develops a bad smell. The use of soap is objectionable because it 20 attacks the silk fiber. Besides it is expensive in use, because the soap which is necessary in the process amounts on an average to as much as 30% of the weight of the raw silk.

25 It has been suggested to use pancreas as a degumming medium for silk. But these experiments have proved a failure as far as practical utility is concerned. My experiments to combine the use of pancreas and that of soap have had no satisfactory results up to this time. Recently I have found, that the failure of this process is due to the fact, that when using enzymes of the pancreas the temperature cannot exceed 40 30 degrees centigrade, because the enzymes are destroyed at higher temperatures, while when degumming the raw silk by means of soap the raw silk is heated to 100 degrees centigrade. I have found that the desired 35 result is obtained when the silk is heated to 100 degrees centigrade after its treatment with the enzyme. In this case the use of soap is not absolutely necessary, but it is advisable to use alkaline salts, because the 40 effect is obtained thereby in a more reliable 45 way. The amount of soap which is necessary in the process is exceedingly small. While heretofore as much as from 30 to 40 per cent. of soap has been used, in my improved process one tenth of this amount is 50 necessary. Also the amount of the enzyme which is necessary in the process is very small. A pancreatin solution of  $\frac{1}{2}$  part per thousand is sufficient. From these data it 55 will be understood that the cost of the proc-

ess is low as compared to the process which is based on the use of soap alone. An important advantage of the new process resides in the fact, that the silk fiber is not in the least affected by the process.

60 The object in heating the silk after it has been treated in a bath of pancreatin is to complete the degumming and to shorten the time for doing so. The sequence of the treatment of pancreatin and the heating 65 may be reversed without departing from the scope of the invention as claimed.

Example: The raw silk is heated a few hours at a temperature of not more than 40 degrees centigrade in an aqueous solution 70 of pancreatin of  $\frac{1}{2}$  part per thousand, whereupon it is heated about 20 or 30 minutes at a temperature of from 90 to 100 degrees centigrade. If desired these steps of the process, viz. the treatment with pancreatin solution and the heating, may be 75 carried out in the reverse order. In both cases the silk is degummed in a satisfactory way. However, it is important, that the steps be not performed at the same time.

80 What I claim and desire to secure by Letters Patent of the United States is:

1. The herein described process of degumming silk and the like, which process comprises the step of subjecting the silk and the like to the action of a pancreatin solution at less than 40° C.; and the step of heating 85 the silk at a higher temperature.

2. The herein described process of degumming silk and the like, which process comprises the step of heating the silk and the like to a temperature higher than 40° C., and the step of subjecting the silk to the action of a pancreatin solution and salts at less than 40° C.

90 3. The herein described process of degumming silk and the like, which process comprises the step of subjecting the silk to the action of a pancreatin solution and alkaline salts at less than 40° C.; and the step of heating the silk and the like to a higher temperature.

100 4. The herein described process of degumming silk and the like, which process comprises the step of subjecting the silk to the action of a pancreatin solution at less than 40° C. and the step of heating the silk at a temperature of 90° to 100° C.

110 5. The herein described process of degumming silk, and the like, which process com-

prises the step of heating the silk at a temperature of 90° to 100° C.; and the step of subjecting the silk to the action of a pancreatin solution and salts at less than 40° C.

5 6. The herein described process of degumming silk and the like, which process comprises the step of subjecting the silk to the action of a pancreatin solution and alkaline salts at less than 40° C.; and the step of

heating the silk at a temperature of 90° to 100° C.

In testimony whereof, I have signed my name to this specification in the presence of two subscribing witnesses.

DR. OTTO ROHM.

Witnesses:

HUGO HANFS,  
ALFRED LIEBIG.